

Nov. 6, 1934.

W. R. WEBSTER

1,980,020

GROUND ROD

Filed Aug. 24, 1931

Fig. 1.



Fig. 2.



Fig. 3.



Fig. 4.



Fig. 5.



Inventor

William R Webster

By  
Rockwell & Bassett  
Attorneys

## UNITED STATES PATENT OFFICE

1,980,020

## GROUND ROD

William R. Webster, Bridgeport, Conn.

Application August 24, 1931, Serial No. 559,027

1 Claim. (Cl. 173—31)

This invention relates to what is commonly known as a ground rod. It is often necessary in connection with electrical wiring to effectively ground certain circuits or parts of circuits. This is true with respect to many electrical installations, and in connection with the operation of overhead electrical circuits for railways and the like, it is necessary to provide at intervals a conducting connection between lightning arresters and other devices and the ground. To effect this end it is convenient to drive into the ground a metal rod, which may be six or eight feet in length. This rod must, of course, comprise conducting material and in the usual instance the top of the rod projects above the ground for several inches when installed, and secured thereto is a wire or suitable conductor which is electrically connected to the device or circuit which it is desired to ground.

It is desirable that the rod so used shall be long enough to extend some distance beneath the surface and preferably to project into the moist layers of earth so that a good ground connection will be had. It is, therefore, necessary that the rod should be as stiff and rigid as possible so that it may be driven into relatively hard or resistant soil without bending or buckling. It is also necessary that the rod should have good electrical conductivity.

One object of this invention is the provision of an improved ground rod which shall be relatively stiff and rigid and which will have good electrical conductivity.

Another object is to provide a strong inexpensive structure in which the rod has a core of ferrous metal and a thin coating of copper or like metal intimately adhering to the core so as to prevent shucking or displacement of the coating relatively to the core and any looseness between said parts.

To these and other ends the invention consists in the novel features to be hereinafter described and claimed.

In the accompanying drawing:

Fig. 1 is an elevational view of a rod which forms the inner portion or core of the completed article;

Fig. 2 is a similar view of the same rod after it has been subjected to a cold drawing operation;

Fig. 3 is a view of the assembled inner core and outer jacket, the assembly having been pointed or reduced at one end;

Fig. 4 shows the parts of Fig. 3 after completion of the operation of drawing the assem-

bly through a die to secure the outer covering or jacket upon the core; and

Fig. 5 is a view illustrating the completed rod.

In manufacturing a ground rod according to my invention, I prefer to use for the inner portion or core of the device a rod 10 shown in Fig. 1, which may be a section of an ordinary hot rolled steel rod. This rod is prepared for cold drawing in the usual or ordinary way, and then drawn in a cold state through a drawing die.

This results in a reduction of the diameter of the rod and also serves to harden it and greatly increase its rigidity and stiffness. The rod which results from this operation is shown at 11 in Fig. 2 of the drawing.

A tube 12 of material of high conductivity, such as copper, for example, having an inside diameter somewhat larger than the cold drawn rod 11 is then slipped over the rod 11 until the end of the tube is substantially flush with that of the rod. This end of the assembled rod and tube is then placed into a suitable pointing device and reduced in size or pointed as shown at 13. This pointing operation results in contracting the outer copper tube upon the rod and renders the end of the assembled tube and rod sufficiently small to be inserted through the opening of a die which is used in the next operation to be performed.

The end 13 of the assembled tube and rod is then inserted through the opening of a suitable drawing die. This pointed end is then grasped by means of draw bench tongs and the assembly is drawn through the die opening. This causes the tube to be reduced in size and to adhere tightly and securely to the surface of the inner steel rod, as shown at 14 in Fig. 4. It will be understood that as the inner steel rod has a relatively smooth exterior surface due to its preparation for the outer covering, the copper tube will be caused to adhere thereto so closely that in effect the two become parts of a unitary structure, that is, there is no danger of any movement of the copper tube or jacket with respect to the core when the rod is driven into the ground.

The rod which has been formed as described is then cut to the required length, which may be six or eight feet, for example, and is sharply pointed at one end, as shown at 15 in Fig. 5. This enables it to be readily driven into the ground when used.

Rods of various diameters may be made by the improved process heretofore described, the diameter, of course, depending upon the diameter of the inner core or steel rod and the thickness of the copper jacket or tubing. In making a  $\frac{5}{8}$  inch

65

70

75

80

85

90

95

100

105

110

rod, for example, I find it convenient to use a hot rolled steel rod approximately  $\frac{5}{8}$  of an inch in diameter. When this rod has been passed through the cold drawing operation and its diameter reduced, as shown in Fig. 2, it will be drawn to approximately .541 inch in diameter. The tube of copper slipped thereon, which is preferably a seamless tube, will have an outside diameter of about  $\frac{3}{4}$  of an inch and have a wall 10 approximately .055 of an inch in thickness. The assembled rod and tube may then be pointed, as shown at 13, so that the outside diameter of the assembly at the pointed end will be slightly less than  $\frac{5}{8}$  of an inch. The assembled rod and tube 15 may then be drawn through a die having a  $\frac{5}{8}$  inch opening so that the outside diameter of the completed rod with its copper jacket will have a diameter of  $\frac{5}{8}$  of an inch. Other sizes may, of course, be made from rods and tubes having corresponding 20 dimensions. The tube of copper is quite thin, having a wall many times less thick than the diameter of the core, as only a thin outer shell of highly conductive metal is required, and on the other hand the reinforcement 25 imparted by the hardened steel core is of such importance that this core should be of comparatively large diameter in order to give the article the requisite mechanical strength.

It will be apparent that the finished ground 30 rod shown at 16 in Fig. 5 is of composite structure having an inner rigid and stiff core of relatively hard material and an outer covering or jacket of high conductivity. The union between the outer covering and the core will be of such

a character due to the method of manufacture that the tube and core will adhere tightly together and will to all intents and purposes be one and the same structure. It will be understood that when the tube is drawn upon the rod which forms the core, it will be forced or contracted upon the rod with considerable pressure so that the metal of the inner surface of the tube and the metal of the outer surface of the rod will become interengaged, i. e., with one extending into minute 35 cavities of the other, thus binding the parts securely together.

While I have shown and described a preferred embodiment of my invention and a preferred method of manufacturing the same, it will be understood that it is not to be limited to all of the details or steps described, but modification and variation may be resorted to within the spirit of the invention and within the scope of the appended claim.

What I claim is:

A ground rod for connecting electrical apparatus to ground comprising a cold drawn core of relatively strong metal, said metal being a ferrous metal, and a cold drawn outer coating of 100 weaker but more highly conductive metal conforming closely to the core, the wall of said coating being quite thin as compared to the diameter of said core and the inner surface of the coating being intimately engaged with and entering 105 minute cavities of the surface of the core to form a substantially unitary structure, said rod having a conical end.

WILLIAM R. WEBSTER.

35

110

40

115

45

120

50

125

55

130

60

135

65

140

70

145

75

150